

1

2,758,972

## ENGINE PRESERVATIVE OILS

William H. Brugmann, Jr., Milltown, Leonard E. Moody, Cranford, and Max W. Hill, Westfield, N. J., assignors to Esso Research and Engineering Company, a corporation of Delaware

No Drawing. Application May 27, 1955,  
Serial No. 511,788

11 Claims. (Cl. 252—33.4)

This invention relates to lubricating oils and methods of compounding them. It particularly relates to engine preservative oils having effective anti-rusting properties needed under specialized conditions.

This application is a continuation-in-part of copending application S. N. 247,754, filed September 21, 1951, now abandoned.

Engine preservative oils are generally employed as lubricants for new automotive equipment and the like during the shipping period and initial breaking-in period. Therefore, such oils must not only meet the requirements expected of engine lubricants for conventional use but also must have versatile rust preventive properties to protect the equipment under a wide variety of corrosive influences. For example, new equipment is susceptible to corrosion by inorganic acids such as HBr formed in the combustion of leaded gasolines. In addition, the engine may encounter corrosion by moisture and aqueous solutions of electrolytes such as sea water or by various other types of corrosive reagents that may come into contact with the metal parts. The oils should also have good detergency properties and inhibit the corrosion of bearings. Prior art lubricating oil formulations may meet one or two of the rigid requirements imposed upon oils used in such service, but do not possess the versatility required when the oils are used in relatively new engines subjected to rather extreme conditions.

It has been found that an unexpectedly superior lubricant from the standpoint of good engine performance and versatile anti-corrosive properties is obtained by compounding with the oil base stock at least four different components, each component cooperating in eliminating or minimizing undesirable characteristics of the oil. These components include an oil-soluble metal salt of an alkylated phenol sulfide, both an alkaline earth metal and an alkali metal oil-soluble petroleum sulfonate, and an oil-soluble aliphatic alcohol. All of these components must be present in the composition to attain the desired degree of protection against corrosion and to provide an oil having the desired detergency characteristics. It is usually desirable to add to the oil a bearing corrosion inhibitor such as  $P_2S_3$  treated terpenes, sulfurized terpenes, thiocarbamates, phenothiazines, xanthates, etc.

The oil-soluble metal salts of the alkyl phenol sulfides useful in the present invention are well known as being effective detergents and sludge dispersers for lubricating oils. Oil-soluble compounds of the phenol sulfide with metals such as sodium, potassium, aluminum, tin, zinc, cobalt, nickel, barium and the like may be used. The preparation of calcium salts of this type and their use in lubricants is disclosed in Mikeska patent, U. S. 2,362,289. The preparation of barium salts is described in the Winning patent, U. S. 2,362,291; the magnesium salts in the McNab patent, U. S. 2,362,292; and mixed alkaline earth salts containing two different

2

alkaline earth metals are described and claimed in U. S. 2,480,664 to McNab, McNulty and Cross.

The alkaline earth metals including calcium, barium, and strontium, are the preferred metals. The presence of at least one alkyl group on the benzene nucleus is desired to impart oil solubility to the composition, the alkyl group containing from about 4 to 12, preferably about 6 to 9, carbon atoms. The alkyl group may be straight or branched chain and includes, for example, such alkyl groups as amyl, hexyl, heptyl, iso-octyl, tert-octyl, nonyl (a polyethylene trimer), decyl, lauryl, etc. Although the invention is not limited to compounds having a definite number of sulfur atoms interconnecting benzene nuclei, compounds containing from 1 to 4 sulfur atoms are preferred. The salts may contain an equivalent of about one mol of metal for each pair of phenol radicals in the compound or may contain up to one mol of metal per phenol radical to form basic, high metal-content salts.

The term "oil-soluble metal salt of the alkyl phenol sulfide" as used herein refers broadly to the single and mixed salts of the various phenol sulfides, as well as to the basic form of these sulfides. As a general rule, the phenol sulfide is added to the composition of the present invention in amounts ranging from about 0.4 to 5% by weight, preferably from 0.5 to 1.0% by weight, of the total composition. Percentages of from 0.6 to 0.91% by weight have been found to be particularly advantageous.

The oil-soluble petroleum sulfonates used in the present invention are the salts of oil-soluble or so-called "mahogany" acids and are prepared by procedures well known to the art. Sodium sulfonate is the preferred alkali metal sulfonate, but potassium and lithium sulfonates may be used. The alkali metal sulfonates will generally have a molecular weight in the range of about 350 to 700.

The alkaline earth metal salts of oil-soluble petroleum sulfonates are preferably the calcium salts although the magnesium, strontium and other alkaline earth metals may be employed. Particularly advantageous also are alkaline earth metal petroleum sulfonates having an excess rather than a stoichiometric amount of polyvalent metal salt added to the sulfonic acid in the preparation step. Such sulfonates may be prepared by the procedure described in U. S. 2,467,176 to Zimmer, Carlson and Duncan. Such sulfonates may be referred to as basic alkaline earth metal oil-soluble petroleum sulfonates. The term "oil-soluble, alkaline earth metal petroleum sulfonates" as used in the present specification and claims refers to both of the above general types of alkaline earth metal sulfonates. The alkaline earth metal sulfonates may vary in molecular weight from about 750 to as high as 1100, although preferably the molecular weight range is from about 800 to 1000. Each type of sulfonate is used in the finished composition in amounts ranging from about 0.4 to 10 wt. percent, but preferably in the range of 0.4 to 1 wt. percent. Percentages of 0.45 to 0.87 wt. percent alkali metal sulfonate and 0.52 to 0.76 wt. percent alkaline earth metal sulfonate have been found to be particularly advantageous. The weight ratio of alkaline earth to alkali metal sulfonate is maintained in the range of about 0.4:1 to 3:1, preferably about 0.6:1 to 1.7:1.

The high molecular weight aliphatic alcohols used in the practice of the present invention should be soluble in low concentrations in the lubricant. They should have at least 7 carbon atoms and preferably no more than 20 carbon atoms. Those having from about 8 to 18 carbon atoms are generally preferred. The saturated straight or branched chain aliphatic alcohols such as octyl, lauryl, cetyl, stearyl, and the like, may be used,

The corresponding olefinic alcohols such as oleyl and the like are also suitable. Mixed naturally occurring alcohols such as the "Lorols" (coconut oil alcohols, C<sub>8</sub> to C<sub>18</sub>, average about C<sub>12</sub>), wool fat which contains substantial amounts of alcohols having 16 to 18 carbon atoms, sperm oil containing a high percentage of cetyl alcohol, and the like may be used. The aliphatic alcohols prepared synthetically by various chemical processes are suitable such as, for example, alcohols produced by oxidation of petroleum hydrocarbons such as paraffin wax, petrolatum and the like which occur in the proper molecular weight range. Particularly advantageous are the alcohols produced by oxonation of olefins, such as polymers and copolymers of propylene and butylenes, with carbon monoxide and hydrogen by the well known Oxo process. Such alcohols, known as "Oxo alcohols," are generally branched chain, saturated aliphatic alcohols. Mixtures of two or more of the above alcohols may be used.

Although the alcohols, when used alone in the oil, are generally quite ineffective for inhibiting metal corrosion by inorganic acids, they are surprisingly effective for this purpose when used in combination with the other ingredients. Corrosion inhibiting amounts of the alcohols are generally rather low. About 0.3 to 2.0 wt. per cent, preferably about 0.4 to 1.5 wt. per cent, of the alcohol is used in the present compositions. The alcohol may be added up to the limit of its solubility in the oil in some cases, but preferably no more than about 2.5 to 3% by weight will be added to the finished composition. The effectiveness of the alcohol used for preventing rusting will vary with its molecular weight, and higher concentrations of high molecular weight alcohols will usually be required than is the case with lower molecular weight alcohols. It is generally preferred that the ratio of average number of carbon atoms in the alcohol to weight per cent concentration of alcohol in the blend be about 9 to 20, preferably about 9 to 17.

In the range of 0.2 to 2.0 wt. per cent of a sulfur-bearing compound, such as an alkyl thiuram disulfide, sulfurized terpenes and the like may be used in the composition as an inhibitor to protect the surfaces of metal bearings from corrosion.

The invention will be further illustrated in the following examples:

#### EXAMPLE I

A series of blends was prepared employing an SAE 30-grade motor oil base stock derived from a solvent extracted, Mid-Continent crude fraction compounded

50

ium). The calcium petroleum sulfonate used in the blends had an average molecular weight of about 950. The sodium petroleum sulfonate used in the blends had an average molecular weight of about 480. C<sub>8</sub> branched-chain, aliphatic alcohols, prepared by the catalytic oxonation of C<sub>7</sub> olefins with carbon monoxide and hydrogen, were used. In addition, the blends in some cases contained sulfurized dipentene and butyl thiuram disulfide as bearing corrosion inhibitors.

The blends were subjected to various corrosion tests. Humidity cabinet life was determined by coating standard steel panels with the blend and placing the panels in a cabinet maintained at a temperature of 100° F., and a relative humidity of 100%. The time in hours required to rust the panels in the cabinet is termed the humidity cabinet life. This test gives a measure of the protection afforded metal surfaces by the engine preservative oils when equipment is used in humid atmosphere.

The blends were tested by the so-called "sea water corrosion test" which is a measure of the extent to which metal surfaces are protected from corrosion by sea water spray when using various preservative oils. In this test, three metal test panels were immersed in the test oil for one minute, and the panels then were suspended in air for 20 hours at room temperature (77° F.). The panels were then suspended in a standard synthetic sea water solution containing various inorganic salts for 20 hours at room temperature. The panels were then cleaned and rated. To pass the test, at least one of the panels must be absolutely free from corrosion and at least one of the other panels must have no more than three small corroded spots. Otherwise, the oil is rated as failing the test.

The blends were also subjected to the HBr corrosion test which indicates the protection afforded metal surfaces by the oils against inorganic acids such as HBr formed in engines by combustion of gasolines containing tetraethyl lead and a lead scavenging agent (usually a bromo-organic compound). Two metal test panels were immersed in an 0.1 wt. per cent aqueous solution of hydrobromic acid for one second. The panels were then immersed in and removed from the test oil a total of 12 times during a period of one minute and then suspended in the air for 4 hours at room temperature. They were then cleaned and rated for corrosion. For an oil to pass the test, one of the panels must be absolutely free of corrosion and the other must have no more than three small corroded spots.

The results of the tests are shown in Table I below:

Table I.—Additives used in SAE 30 base stock

| Blend No. | Barium tert-octyl phenol sulfide (wt. percent) | Ca sulf. (wt. percent) | Na sulf. (wt. percent) | Wt. ratio Ca to Na sulfonate | C <sub>8</sub> alcohol (wt. percent) | Sulfurized dipentene (wt. percent) | Humidity cabinet life (hrs.) | Sea water corr. | HBr corr. test |
|-----------|------------------------------------------------|------------------------|------------------------|------------------------------|--------------------------------------|------------------------------------|------------------------------|-----------------|----------------|
| A         |                                                |                        |                        |                              | 0.6                                  |                                    |                              | Fail            | Fail           |
| B         | 1.37                                           | 2 <sup>1</sup> 0.62    |                        |                              |                                      |                                    | <3                           | do              | Fail           |
| C         | 1.37                                           | 2 <sup>1</sup> 0.62    | 0.5                    | 1.25                         |                                      |                                    | 200                          | Pass            | Do             |
| D         | 1.37                                           | 2 <sup>1</sup> 0.62    | 1.0                    | 0.62                         |                                      |                                    | 312                          | do              | Do             |
| E         | 1.37                                           | 2 <sup>1</sup> 0.62    |                        |                              | 0.6                                  |                                    | <3                           | do              | Pass           |
| F         | 1.083                                          | 2 <sup>1</sup> 0.76    | 0.43                   | 1.77                         |                                      |                                    | 216-240                      | do              | Fail           |
| G         | 1.083                                          | 2 <sup>1</sup> 0.76    | 0.43                   | 1.77                         |                                      | 0.6                                | 216-240                      | do              | Do             |
| H         | 1.081                                          | 2 <sup>1</sup> 0.75    | 0.45                   | 1.67                         | 1.04                                 |                                    | 200-240                      | do              | Pass           |
| I         | 1.060                                          | 2 <sup>1</sup> 0.76    | 0.73                   | 1.04                         |                                      | 0.3                                | 240-288                      | do              | Fail           |
| J         | 1.060                                          | 2 <sup>1</sup> 0.76    | 0.73                   | 1.04                         | 0.6                                  | 0.3                                | 312                          | do              | Pass           |
| K         | 1.091                                          | 2 <sup>1</sup> 0.52    | 0.87                   | 0.60                         | 0.4                                  | 0.24                               | 240                          | do              | Do             |

<sup>1</sup> Basic barium tert-octyl phenol sulfide.

<sup>2</sup> Calcium sulfonate (5.0 wt. percent calcium).

<sup>3</sup> Basic Ca sulfonates (6.5 wt. percent calcium).

<sup>4</sup> Ratio of No. of C atoms in alcohol to wt. percent conc. of alcohol—about 13.

<sup>5</sup> Butyl thiuram disulfide used instead of sulfurized dipentene.

with various combinations of additives. The alkaline earth metal salt of the alkyl phenol sulfide used in the blends was either barium tert-octyl phenol sulfide (containing 21.7 wt. per cent barium) or basic barium tert-octyl phenol sulfide (containing 30.1 wt. per cent bar-

75

ium) and calcium sulfonate had a very low humidity cabinet life (blend B), but the addition of sodium sulfonate to the oil produced a finished blend having a satisfactory humidity cabinet life (blends C, D, and F). None of

these blends, however, passed the HBr corrosion test. When  $C_8$  alcohols were added to a blend containing barium tert.-octyl phenol sulfide and calcium sulfonate, the final blend had a low humidity cabinet life, but passed the HBr corrosion test (blend E). When  $C_8$  alcohols were added to blends containing barium tert.-octyl phenol sulfide, calcium sulfonate, and sodium sulfonate, the final blend had a high humidity cabinet life and passed both the sea water corrosion and HBr corrosion tests. The addition of a bearing corrosion inhibitor such as sulfurized dipentene made no significant difference in improving the oil from the standpoint of either humidity cabinet life or HBr corrosion tests.

It is, therefore, seen from the results obtained on the above blends that both an alkaline earth and an alkali metal petroleum sulfonate must be present in the finished blend to obtain a satisfactory humidity cabinet life. Both a salt of an alkyl phenol sulfide and an alkaline earth metal petroleum sulfonate must be used in the blend to obtain desired detergency characteristics. The presence of an alcohol along with the other components was found to be essential to impart the desired degree of protection to the oil against corrosion by acids such as HBr.

#### EXAMPLE II

Blend K from Example I was also evaluated in a Lauson engine to determine its bearing corrosion inhibition and detergency properties. A sample of the SAE 30 grade oil per se was tested for purposes of comparison. The tests were conducted for 25 hour periods, the engine being operated at 1800 R. P. M. with a 1.5 indicated kilowatt load, 300° F. oil temperature and 295° F. water jacket temperature. The oils were then rated on a demerit system wherein a perfectly clean surface is given a rating of 0, while a rating of 10 is given the worst condition that can be expected of that surface. The loss in weight of the copper-lead bearings during the test was determined. Results are shown below:

| Lubricant  | Piston varnish demerit | Bearing weight loss, (mgs./bearing) |
|------------|------------------------|-------------------------------------|
| SAE 30 oil | 5.50                   | 100                                 |
| Blend K    | 0.88                   | 16                                  |

The detergency and bearing corrosion properties of blend K are seen to be quite satisfactory.

#### EXAMPLE III

A series of blends was prepared using the base oil of Example I. In each case the blends contained 0.81 wt. per cent of basic barium tert.-octyl phenol sulfide, 0.75 wt. per cent basic calcium sulfonate, and 0.45 wt. per cent sodium sulfonate, the latter ingredients being identical to the compounds used in preparing the blends of Example I. These blends, containing different concentrations of various alcohols, were then tested for HBr corrosion characteristics in accordance with the above described procedure. The data are as follows:

| Blend No. | Alcohol used in blend               |                            | Ratio, No. of C atoms in alcohol to alcohol conc. | HBr corr. test |
|-----------|-------------------------------------|----------------------------|---------------------------------------------------|----------------|
|           | Type                                | Concentration, wt. percent |                                                   |                |
| L         | $C_{13}$ "Oxo" alcohol <sup>1</sup> | 0.6                        | 21                                                | Fail.          |
| M         | do                                  | 1.0                        | 13                                                | Pass.          |
| N         | $C_{17}$ alcohols                   | 0.6                        | 28                                                | Fail.          |
| O         | do                                  | 1.0                        | 17                                                | Pass.          |
| P         | "Lorol B" alcohols <sup>2</sup>     | 1.0                        | 13                                                | Borderline.    |
| Q         | do                                  | 1.5                        | 9                                                 | Pass.          |

<sup>1</sup> Branched chain alcohols prepared by conventional catalytic oxonation of  $C_{12}$  polymer (from low molecular weight olefins) with CO and  $H_2$ .

<sup>2</sup>  $C_{10}$ - $C_{15}$  alcohols, average about  $C_{12.5}$  alcohols.

Higher concentrations of the high molecular weight alcohols ( $C_{12}$ - $C_{20}$ ) are generally required to prevent rusting than is required in the case of lower molecular weight alcohols.

- 5 The lubricating oil base stocks used in the compositions of this invention may be straight mineral lubricating oils or distillates derived from various crudes, or various blended oils may be employed as well as de-asphalting residuals. The oils may be refined by conventional methods such as by clay treating, solvent extraction, and the like. Hydrogenated oils or white oils may also be used. Synthetic oils prepared by the polymerization of olefins, by the reaction of oxides of carbon with hydrogen, or by the hydrogenation of coal or its products may be employed. Certain animal, vegetable or fish oils or their hydrogenated products may be employed, either alone or in a mixture with mineral oils. The ester- and ether-type synthetic lubricants may also be employed advantageously.
- 10 Examples of other operable synthetic oils include ether alcohols such as those corresponding to the general formula



25 wherein R is an alkyl group, for example, butyl, n is an integer from 1 to 5, and x is an integer greater than 1; esters of monobasic carboxylic acids totaling 20 to 130 carbon atoms, such as those  $C_4$  to  $C_{18}$  aliphatic acids with  $C_4$  to  $C_{18}$  aliphatic alcohols, the  $C_4$  to  $C_{18}$  radicals including the butyl, isobutyl, hexyl, octyl, iso-octyl, 2-ethyl hexyl, nonyl, decyl, lauryl, stearyl and similar radicals; diesters of dibasic acids such as adipic or sebacic acids with monohydric alcohols such as hexyl, octyl, 2-ethyl hexyl or higher alcohols; esters of polyethylene glycols with  $C_8$  to  $C_{18}$  branched chain carboxylic acids; complex esters of polybasic carboxylic acids, polyhydric alcohols, monobasic acids and/or monohydric alcohols, such as the well known glycol-centered or dibasic acid-centered complex esters; phosphoric acid esters or thioesters of aliphatic alcohols or mercaptans of up to 18 carbon atoms; halocarbon oils such as the polymers of chlorotrifluoro ethylenes like chlorotrifluoroethylene; organo-siloxanes; sulfide esters; organic carbonates; mercaptals; formals; etc.

30 40 The lubricating oils may vary considerably in viscosity and other properties, depending on the particular use for which they are desired, but they will usually range from about 35 to 150 seconds Saybolt Universal viscosity at 210° F. In preparing the compositions of the invention major proportions constituting from about 70 to 98.5 wt. per cent, preferably about 85 to 97 wt. per cent, of mineral and/or synthetic lubricating oils are employed.

45 50 It is also within the scope of the present invention to add other agents as may be needed. Such additives include dyes, pour point depressors, heat thickened fatty oils, sludge dispersers, antioxidants, viscosity index improvers, oiliness agents, anti-wear agents and the like.

What is claimed is:

- 60 65 70 75 1. A composition of matter consisting essentially of a major proportion of a lubricating oil, from 0.5 to 1.0 wt. per cent of basic barium tert.-octyl phenol sulfide, 0.4 to 1.0 wt. per cent of basic calcium petroleum sulfonate, 0.4 to 1.0 wt. per cent of sodium petroleum sulfonate, and 0.3 to 2.0 wt. per cent of an aliphatic alcohol containing from 7 to 20 carbon atoms per molecule and a ratio of the number of carbon atoms in said alcohol to the weight per cent concentration of said alcohol in the range of about 9 to 20.
2. The composition of matter of claim 1 wherein said aliphatic alcohol contains from 8 to 18 carbon atoms per molecule and said ratio of the number of carbon atoms in said alcohol to the weight per cent concentration of said alcohol is in the range of about 9 to 17.
3. The composition of matter of claim 1 which includes

a corrosion inhibiting amount of a sulfur-containing compound selected from the group consisting of sulfurized dipentene and butyl thiram disulfide.

4. The composition of matter of claim 1 wherein said lubricating oil is a mineral lubricating oil.

5. An engine preservative oil consisting essentially of a major proportion of a mineral lubricating oil, 0.6 to 0.91 wt. per cent of basic barium tert.-octyl phenol sulfide, 0.52 to 0.76 wt. per cent of basic calcium petroleum sulfonate, 0.45 to 0.87 wt. per cent of sodium petroleum sulfonate, and 0.4 to 1.5 wt. per cent of an aliphatic alcohol containing from 8 to 18 carbon atoms per molecule and a ratio of the number of carbon atoms in said alcohol to the weight per cent concentration of said alcohol in the range of about 9 to 17.

6. The engine preservative oil of claim 5 wherein said aliphatic alcohol is a branched chain, saturated aliphatic alcohol.

7. The engine preservative oil of claim 5 wherein said aliphatic alcohol is a straight chain, saturated aliphatic alcohol.

8. An engine preservative oil consisting essentially of a major proportion of a mineral lubricating oil, 0.81 wt. per cent basic barium tert.-octyl phenol sulfide, 0.75 wt. per cent of basic calcium petroleum sulfonate, 0.45 wt. per cent of sodium petroleum sulfonate and 0.6 to 1.5 wt. per cent of an aliphatic alcohol containing from 8 to 18 carbon atoms per molecule and a ratio of the number of carbon atoms in said alcohol to the weight per cent concentration of said alcohol in the range of about 9 to 17.

9. An engine preservative oil consisting essentially of a major proportion of a mineral lubricating oil, 0.6 wt. per cent of basic barium tert.-octyl phenol sulfide, 0.76 wt. per cent of basic calcium petroleum sulfonate, 0.73

wt. per cent of sodium petroleum sulfonate, 0.6 wt. per cent of a branched chain saturated aliphatic alcohol containing 8 carbon atoms per molecule and 0.3 wt. per cent of sulfurized dipentene.

10. An engine preservative oil consisting essentially of a major proportion of a mineral lubricating oil, 0.91 wt. per cent of basic barium tert.-octyl phenol sulfide, 0.52 wt. per cent of basic calcium petroleum sulfonate, 0.87 wt. per cent of sodium petroleum sulfonate, 0.4 wt. per cent of a branched chain saturated aliphatic alcohol containing 8 carbon atoms per molecule and 0.24 wt. per cent of butyl thiram disulfide.

11. A composition of matter comprising essentially a major proportion of a lubricating oil, from 0.5 to 1.0 wt. per cent of a basic alkaline earth metal alkyl phenol sulfide, said alkyl group containing from about 4 to 12 carbon atoms, 0.4 to 1.0 wt. per cent of basic calcium petroleum sulfonate, 0.4 to 1.0 wt. per cent of sodium petroleum sulfonate, and 0.3 to 2.0 wt. per cent of an aliphatic alcohol containing from 7 to 20 carbon atoms per molecule and a ratio of the number of carbon atoms in said alcohol to the weight per cent concentration of said alcohol in the range of about 9 to 20.

25 **References Cited in the file of this patent**

UNITED STATES PATENTS

|           |               |               |
|-----------|---------------|---------------|
| 2,409,726 | Winning       | Oct. 22, 1946 |
| 2,412,633 | Schwartz      | Dec. 17, 1946 |
| 2,412,634 | Schwartz      | Dec. 17, 1946 |
| 2,418,894 | McNab et al.  | Apr. 15, 1946 |
| 2,560,202 | Zimmer et al. | July 10, 1951 |

FOREIGN PATENTS

|         |               |                |
|---------|---------------|----------------|
| 715,407 | Great Britain | Sept. 15, 1954 |
|---------|---------------|----------------|